

## UNITED STATES PATENT OFFICE

1,924,457

## BRIQUETTE AND BINDER FOR THE SAME

Isidor Rosenwald, Parksville, N. Y., assignor of  
one-third to Mildred Belous, Brooklyn, N. Y.,  
and one-tenth to Benjamin Kirschstein, New  
York, N. Y.

No Drawing. Application July 2, 1932  
Serial No. 620,728

8 Claims. (Cl. 44—18)

My invention relates to briquettes and binders for the same. More particularly my invention relates to coal briquettes of relatively high porosity having their constituent particles firmly bonded and adhering together without any danger of crumbling or disintegration after their formation.

In the ordinary type of coal or other fuel briquette, the constituent coal particles are bonded together by agents such as tar, asphalt, pitch, resins, and the like. In all such cases, a relatively high proportion of binding agent must be used in order to obtain a fuel briquette of the desired quality. The binding agent furthermore in such type of briquette has the tendency of entirely coating the coal particles so that when such briquettes are used as fuel, the binding agent must be first burned before the coal itself is affected. Such a briquette being also compressed, has its ingredients compacted together without any air spaces or interstices between the coal particles, thus requiring more oxygen for combustion and incidentally involving the use of more initial burning agent to kindle the briquette.

It is an object of my invention to provide a relatively porous briquette for fuel purposes which is easy and very economic to manufacture.

Another object of my invention is to provide a coal briquette made of relatively cheap raw materials and having a high fuel or combustion value.

A further and more particular object of my invention is to provide a water-proof briquette having coal particles with a small proportion of strongly adhering bonding material, which is strong and resistant to any disintegrating and crushing actions to which briquettes are normally subjected in metallurgical and like operations.

One other object of my invention is to provide a coal briquette in which the particles of coal dust are tenaciously held together in spaced relation by a bonding agent and which has air interstices or spaces between the particles to permit efficient and complete combustion of the particles with maximum thermal utilization thereof.

Other objects and features will be more apparent in the following description and claims:—

In the preferred embodiment of my invention, the ingredients are easy to mix, requiring little or no skill and the operation to obtain the desired briquette requires little time and is very economical.

According to my invention in its preferred form, I employ coal of any kind generally used as a fuel, with a binding agent consisting of lime (CaO) and skimmed powdered milk and water.

The improved briquette is constructed as follows:

Five grams of powdered skimmed milk are thoroughly mixed with an equal quantity of lime (calcium oxide). To this mixture is added a sufficient quantity of water to form a paste of strongly adhering properties. The water slakes the lime and partly dissolves the milk powder to permit a chemical action between the slaked lime and the powder.

Once the paste has been formed, a pound of coal in properly comminuted form is added in small quantities at a time and thoroughly incorporated until a uniform mixture is obtained of the coal particles and the paste. It is to be understood, however, that the quantity of water required does not adversely affect the composition since it is subsequently driven off to obtain a water free briquette. Also, I may add more water during the mixing of the coal particles if desired in order to obtain a composition of desired consistency.

Once the mixture is made uniform, it is compressed and then dried in any well known manner to form a strong, very easily made, and cheap coal briquette from raw materials which are easily and readily obtainable in large quantities. The resultant briquette is waterproof and highly resistant to disintegration.

In the formation of the adhesive binding agent, the lime, upon addition of the water, forms slaked lime which combines with the skimmed powdered milk. There is formed an adhesive paste of apparently colloidal character which upon addition of the coal particles physically combines with them. Upon drying the composition, the water therein is driven off and the particles are held together in spaced apart relation by an adhesive in the whole mass of the resulting briquette. The water in drying or evaporating causes the formation of air spaces or interstices of microscopic character, while the adhesive does not enclose the whole body of the particles but apparently links the particles together, leaving the major portion of the body of the particles exposed to air. This is a highly desirable feature particularly when the briquettes are packed in a furnace and the amount of air supplied to the briquettes to aid

combustion must be regulated, for example in coking and like processes.

The briquette embodying the present invention is made from raw materials which are easily obtainable. Also, the briquette has a high crushing strength, not readily disintegrating. It moreover has a high B. t. u. and is easily combustible, due to its somewhat porous internal structure. The briquette also is easy 10 to make and well adapted for use in any type of furnace or stove.

While I have disclosed a preferred embodiment of my invention, it is to be understood that various modifications as to ingredients and 15 proportions may be made without being limited to the embodiment herein disclosed.

This application is a continuation in part of my application now pending in the U. S. Patent Office under Serial No. 500,423, filed December 20 5, 1930, Patent No. 1,891,450 granted December 20, 1932.

In this application, I have described a binder of chalk and pot cheese, and water, the proportions of which are: three grams of chalk and 25 three grams of cheese, per pound of coal dust. Cheese and chalk are first mixed in water to form a paste which is then combined with the coal dust.

The chalk ( $\text{CaCO}_3$ ) of that application is now 30 represented by lime ( $\text{CaO}$ ) and the constituents of the pot cheese, find their counterpart in skimmed powdered milk. The present invention is inclusive then of calcium-oxygen-containing compounds combined with the ingredients of the 35 pot cheese or skimmed milk powder, both having non-acid caseins. The  $\text{CaCO}_3$ , when used, is dried with the pot cheese and thereby the  $\text{CaCO}_3$  calcined in which  $\text{CO}_2$  comes off and  $\text{CaO}$  remains. The constituents of pot cheese and 40 skimmed milk powder, are essentially non-acid casein, so that the non-acid casein and alkaline  $\text{CaO}$ , chemically combine to form a semi-colloidal product. This product having been thoroughly mixed in the presence of air and water, 45 and when thus applied to coal dust, the product is plastic and slightly wetted, and upon the drying of the water, the product becomes porous

50

55

60

65

70

75

and filled with air chambers, the walls of which again have openings to permit the influx of air during combustion. The walls themselves form links or bridges holding one dust particle to the other.

80

The links and connecting struts form bonds for the separated coal particles, the bonds resembling generally a honeycomb-like structure, so that the coal particles are air-enclosed, and upon ignition, readily form  $\text{CO}$ , and due to the preponderance of air inflow through the porous linkage walls to the ignited carbon particle, quickly form  $\text{CO}_2$ , or substantially perfect combustion.

85

I claim:

1. A briquette having particles of fuel material, lime and skimmed milk.

90

2. A porous briquette for fuel purposes, comprising particles of fuel material, and a bonding agent containing skimmed milk.

95

3. A combustible porous briquette, comprising particles of fuel material and an adhesive agent containing lime, and skimmed milk for holding said particles in spaced apart relation.

4. A fuel briquette, comprising coal particles, skimmed milk powder, lime and water.

100

5. A fuel briquette, comprising coal dust, skimmed milk powder and slaked lime, and having a microscopic, substantially porous structure.

105

6. A fuel briquette, comprising one pound of pulverized fuel material, five grams of powdered skimmed milk, five grams of lime, and sufficient water to form an adhesive action between the fuel material and the milk and lime.

110

7. The process of making fuel briquettes consisting of mixing powdered skimmed milk with lime, adding water to the resultant mixture to form a paste, then adding pulverized fuel material to the paste with constant stirring to form a uniform mass, compressing the mass, and finally drying.

115

8. A briquette composed of coal dust particles, and a binder of calcium-oxygen-containing compounds and constituents of fat-free milk products.

120

ISIDOR ROSENWALD.

125

130

135

140

145

150